

1

3,518,085

## LITH-TYPE EMULSIONS CONTAINING A POLYALKYLENEOXY POLYMER AND A 3-PYRAZOLIDONE DEVELOPING AGENT

Kirby M. Milton and Charles A. Goffe, Rochester, N.Y., assignors to Eastman Kodak Company, Rochester, N.Y., a corporation of New Jersey

No Drawing. Filed Sept. 23, 1965, Ser. No. 489,736

Int. Cl. G03c 5/24, 1/28, 1/04

U.S. Cl. 96—66.3

23 Claims

### ABSTRACT OF THE DISCLOSURE

High contrast photographic emulsions in which the silver halide comprises at least 50% silver chloride are improved by the addition of a polyalkyleneoxy polymer and a 3-pyrazolidone silver halide developing agent. Further improvement is obtained by the incorporation of a vinyl polymer and an onium salt.

This invention relates to high-contrast, silver-halide-sensitized photographic materials for graphic arts use and particularly to lith-type silver halide emulsion layers of improved physical and photographic properties.

In the photomechanical arts, photographic films capable of providing high image contrast and good dimensional stability with varying temperature and humidity are required for the preparation of the line and halftone film intermediates which are used in making printing plates. In reproducing continuous tone material, it is customary to make a halftone photographic intermediate, usually a film negative, in which the gradations in tone are represented by differing sizes of dots of uniform density. The shape, density and uniformity of the halftone dots are closely correlated to the quality of the resulting picture.

Most lith films are processed in hydroquinone-type developers which contain relatively low concentrations of sulfite ion. The dot quality and the development contrast obtained in processing lith emulsions in such developers can be improved by processing in the presence of certain water-dispersible polymers containing substantial proportions of ethylene oxide units, such as polyethylene oxides, their terminally substituted derivatives, block copolymers containing ethylene oxide units, etc. These can be added either to the photographic element or the developing solution or both.

It is further advantageous to use as part of the colloid binder for lith type emulsions a colloid-compatible vinyl polymer, the presence of which improves the dimensional stability of the resulting lith film.

The marked improvement resulting from the use of the ethylene oxide polymer on the contrast and dot quality of the emulsion and that of the vinyl polymers on the dimensional stability of the element may result in certain unwanted effects on other properties such as decreasing the developing rate, impairing the emulsion speed, and narrowing the development latitudes.

There is accordingly a need for a lith film system which will provide the advantages afforded by the above two types of addenda without the possibility of detrimental

2

results and which will produce measurable and simultaneous improvements in (1) physical properties, e.g., dimensional stability and emulsion hardness, (2) photographic properties, e.g., exposure latitude, sensitivity, contrast, line and dot quality, and (3) processing characteristics, e.g., development rate and development latitude.

We have found a method of overcoming the undesirable side effects of adding polymers to the gelatin of lith-type emulsions without impairing their beneficial action.

It is an object of this invention to provide a photographic lith-type silver halide sensitized film of high dimensional stability, which yields high contrast, excellent dot quality, high emulsion speed, which develops uniformly in short developing times, and which shows superior exposure and development latitude.

It is a further object to provide lith-type films containing a compound which reduces the adverse effect of prolonged development induction times which may be required when certain vinyl polymers are used to improve dimensional stability.

It is a further object to provide lith-type films containing a compound which regains the effective photographic speed lost when certain ethylene oxide polymers are used to improve contrast and dot quality.

It is a further object to provide lith-type films containing a compound which produces, synergistically in combination with certain ethylene oxide block copolymers, improved speed, contrast and dot quality.

It is also an object to provide improvements in the development of silver halide images.

It is a further object to provide a photographic lith film with improved properties which can be processed in a simple lith-developer containing a sufficiently high concentration of sulfite ion to provide good resistance to aerial oxidation by the developer.

It is a further object to provide lith-type films containing a compound which reduces the adverse effect on emulsion hardness which may be produced by certain ethylene oxide polymers used to improve contrast and dot quality.

We have accomplished these and other objects which will be apparent from the further disclosures and the claims by adding a 3-pyrazolidone compound to lith-type silver halide sensitized photographic materials containing polymeric addenda for the purpose of improving photographic properties.

Our invention provides an improved photographic lith-type film material comprising a radiation sensitive hydrophilic colloid silver halide emulsion, an alkyleneoxy polymer, and a 3-pyrazolidone.

In one embodiment of this invention an aqueous silver chlorobromoiodide lithographic emulsion containing at least 50% silver chloride and a reduced amount of gelatin is prepared in a manner familiar to those skilled in the art. To this emulsion are then added a gelatin-compatible vinyl polymer, a polyalkyleneoxy compound and a pyrazolidone silver halide developing agent. This preparation is then coated on a suitable film support, dried, sensitometrically exposed, processed in a lith-type developing solution, fixed and dried.

The fine grain silver halide emulsions used to advantage have silver halide crystals preferably containing at least 50 mole percent chloride. The emulsions can be prepared as described by MacWilliam U.S. 2,756,148, issued July

24, 1956. These emulsions may be used without being sensitized, however, it is advantageous to spectrally sensitize them according to methods well known in the art to make them ortho-sensitized or panchromatically-sensitized.

The silver halide is dispersed in hydrophilic colloid materials used as binders, including gelatin, collodion, gum arabic, cellulose ester derivatives, such as, alkyl esters of carboxylated cellulose, hydroxy ethyl cellulose, carboxy methyl hydroxy ethyl cellulose, synthetic resins, such as the amphoteric copolymers described by Clavier et al. in U.S. Pat. 2,949,442, issued Aug. 16, 1960, polyvinyl alcohol, and others well known in the art. Examples of these polymeric gelatin substitutes are copolymers of allylamine and methacrylic acid; copolymers of allylamine, acrylic acid and acrylamide; hydrolyzed copolymers of allylamine, methacrylic acid and vinyl acetate; the copolymers of allylamine, acrylic acid and styrene; the copolymers of allylamine, methacrylic acid and acrylonitrile; alkyl acrylate—acrylic acid copolymers, e.g., copolymers of butyl acrylate—acrylic acid; etc.; and etc.

Useful compatible vinyl polymers include the following:

(1) Copolymers of butylacrylate and acrylic acid such as those disclosed in U.S. Pat. 3,062,674.

(2) Interpolymers of acrylic acid, unsaturated carboxylic acid esters, and sulfobetaines such as those disclosed in U.S. Ser. No. 449,879 filed Apr. 21, 1965, now U.S. Pat. No. 3,411,912.

(3) Interpolymers of alkyl esters of unsaturated carboxylic acid with sulfoesters of unsaturated carboxylic acids such as those disclosed in U.S. Ser. No. 454,683 filed May 10, 1965, now Pat. No. 3,411,911.

(4) Homopolymers of acrylic acid esters, homopolymers of  $\alpha$ -hydrocarbon substituted acrylic acid esters. Copolymers of unsubstituted or substituted acrylic acid esters with other vinyl compounds, containing at least 90% by weight of acrylic acid ester structural units such as those disclosed in British Pats. 955,191 and 961,490.

The vinyl polymers are incorporated in the photographic elements of our invention at quantities ranging from approximately 30 to 80 percent of the total emulsion vehicle. In one embodiment in which a gelatin emulsion is employed, the ratio of gelatin to vinyl polymer ranges from 20:80 to 80:20 parts by weight.

Other vinyl polymers useful in our invention may include those disclosed in U.S. Pats. No. 1,933,052, patented Oct. 31, 1933 and No. 2,140,048, patented Dec. 13, 1938 and U.S. Alien Property Custodian Ser. No. 397,138, published May 11, 1943.

The alkyleneoxy polymers useful in this invention are:

(1) Water-dispersible polyethylene oxides having molecular weights of from approximately 400 to approximately 4,000. Particularly useful polyethylene oxides include the following:

|                           | M.W. |
|---------------------------|------|
| Polyethylene glycol ----- | 400  |
| Polyethylene glycol ----- | 600  |
| Polyethylene glycol ----- | 425  |
| Polyglycol -----          | 1000 |
| Polyglycol -----          | 4000 |

These compounds may be expressed by the general formula:



wherein  $n$  is an integer greater than 10.

Other useful polyglycols include, for example, polyethylene glycol oleyl ether, polyethylene glycol ether, as well as the polyethylene glycols disclosed in U.S. Pats. Nos. 2,531,832, 2,423,549, and 2,886,437.

(2) Water-dispersible alkyleneoxy block copolymers containing at least about 30 percent by weight of ethyleneoxy units. Particularly useful water-soluble block polymers include those block polymers in which the polyoxypropylene chain (or moiety) has an average molec-

ular weight between 800 and 3,000 and in which the polyoxyethylene units constitute from about 10 to about 70 percent by weight of the polymer.

The water-soluble block polymers of polyoxypropylene and polyoxyethylene used to advantage include those represented by the formula:



wherein Y represents an organic radical having a valence of  $x$ , said radical being the residue of an organic compound containing atoms selected from the class consisting of carbon, hydrogen, oxygen, nitrogen and sulfur with  $x$  active hydrogen atoms, such as, the residue of polyhydroxy compounds, e.g., ethylene glycol, 1,2-propanediol, 1,5-pentanediol, 1,2,3-propanetriol, sucrose, etc., the residue of a polybasic acid, e.g., oxalic acid, malonic acid, succinic acid, maleic acid, citric acid, etc., the residue of a polyamine, e.g., ethylenediamine, 1,3-diaminopropylene, etc., the residue of a polyamide, e.g., malonamide, succinamide, etc., the residue of a polythiol, e.g., 1,2-ethylenedithiol, 1,3-propylenedithiol, etc.,  $n$  is an integer greater than 1;  $x$  is an integer greater than 1, so that the values of  $n$  and  $x$  are such that the molecular weight of the said polymer exclusive of Y, E and R is between 800 and 3,000; E represents a polyoxyethylene chain constituting from about 10 to about 70 percent by weight of said block polymer; and R represents the hydrogen atom, an alkyl group having from 1 to 20 carbon atoms, (such as methyl, propyl, decyl, dodecyl, octadecyl, etc.), an alkyl carbonyl group in which the alkyl groups has from 1 to 20 carbon atoms as described above, an aryl carbonyl group, such as, benzoyl, p-methyl benzoyl, etc.

Included among the preferred block polymers are those having the formula:



in which  $b$  represents an integer of from 14 to 42;  $a$  and  $c$  are each integers such that the sum of  $a+c$  has a total of from 4 to 48 and the polyoxyethylene groups constitute between 10 and 70 percent by weight of the block polymer.

The block polymers of Formula II and of Formula I where R represents the hydrogen atom are described in Lundsted U.S. Pat. 2,674,619, issued Apr. 6, 1954 and Lundsted U.S. Pat. 3,022,335, issued Feb. 20, 1962. The block polymers of Formula I in which R is hydrogen are readily converted to compounds where R represents an organic residue by reaction with the appropriate reagent in a suitable inert organic solvent that is preferably anhydrous. For example, alkyl halides, such as alkyl chlorides, alkyl bromides, etc., are used to advantage to replace the terminal hydrogen atom of the block polymer with an alkyl group. Alkyl-p-toluenesulfonates are also used to advantage to place an alkyl group at the end of the block polymers. The appropriate acid chloride or acid anhydride, such as, acetyl chloride, propionyl chloride, stearoyl chloride, benzoyl chloride, acetic anhydride, etc., are used to advantage to prepare block polymers of Formula I in which R is an alkyl carbonyl or an aryl carbonyl group.

(3) Water-dispersible alkyleneoxy block copolymers containing at least about 30 percent by weight of ethyleneoxy units and containing in their main chain up to approximately 15 percent by weight silicone atoms. Particularly useful water-soluble organosilicone polyalkylene-oxide polymers include those disclosed in U.S. Pat. No. 2,917,480, issued Dec. 15, 1959. Polymers used to advantage are of the type which are prepared by reacting a dialkyl siloxane with a compound of the following structure:



wherein Y is the residue of an organic compound containing therein, x active hydrogen atoms, and wherein n is an integer, x is an integer greater than 1, the values of n and x are such that the molecular weight of the compound exclusive of E and R is between 800 and 3,000, and E is a polyoxyethylene chain constituting 10-70% by weight of the compound, R is hydrogen or the residue of an organic compound containing an active hydrogen atom; e.g., alcohols, amines, acids, amides, phenols, etc.

The above alkyleneoxy block copolymers (2 and 3) have molecular weights ranging from approximately 600 to about 10,000.

The alkyleneoxy polymers may be added to the photographic element at any stage in the preparation. They may be added as such or from an aqueous solution or from an organic solvent, e.g., ethanol, but are advantageously added from solutions in water. They are added to the aqueous hydrophilic colloid (either with or without the silver halide) before it is coated. The alkyleneoxy polymers can be used to advantage over a wide range of concentrations. The operable range of concentrations is from 0.01 to 3.00 gram of polymer per mole of silver, while the particularly useful range is from 0.010 to 1.0 gram per mole of silver. The optimum concentration of a given alkylene oxide-containing polymer used in my elements depends upon the results desired, the particular silver halide emulsion, the developer solution, etc., and is readily determined by methods known in the art. The determination of the optimum concentration is preferably made by employing the alkyleneoxy polymer in the silver halide emulsion layer or in an adjacent hydrophilic colloid layer according to the element that is desired.

It is advantageous to add certain onium salts, such as, quaternary ammonium salts, sulfonium salts and phosphonium salts to our light-sensitive emulsions in order to increase the photographic speed without adversely affecting the improved dot quality, contrast and evenness of development. Examples of quaternary ammonium salts include nonyl pyridinium perchlorate, hexoxymethyl pyridinium perchlorate, ethylene bis-dioxymethyl pyridinium perchlorate and others described by Carroll U.S. 2,271,623, issued Feb. 3, 1942, hexadecamethylene 1,16-bis(pyridinium perchlorate), 9,16-diaza-7,18-dioxa-8,17-dioxotetacosane - 1,24 - bis(pyridinium perchlorate), and others of Beavers et al. U.S. 2,944,898, issued July 12, 1960. Other examples include the onium salts of polyoxyalkylenes of Carroll et al., U.S. 2,944,902, issued July 12, 1960, the polyonium salts of Carroll et al. U.S. 2,288,226, issued June 30, 1942, such as bis(lauryl methyl sulfonium p-toluene sulfonate) 1,2-ethane, N,N'-trimethylene dioxymethyl pyridinium perchlorate, etc., the sulfonium salts of Carroll et al. U.S. 2,275,727, issued Mar. 10, 1942, such as, n-decyl dimethyl sulfonium p-toluene sulfonate, n-nonyl dimethyl sulfonium p-toluene sulfonate, etc., and the phosphonium salts of Carroll et al. U.S. 2,271,622, issued Feb. 3, 1942, such as, tetramethylene bis-triethyl phosphonium bromide, lauryltriethylphosphonium bromide, etc.

The onium salts are added to the photographic materials at concentrations ranging from approximately 0.01 to approximately 2.0 gram per mole of silver in the light sensitive emulsions. The preferred range is from approximately 0.035 gram to approximately 0.65 gram per mole of silver.

The use of the onium compound alone does not result in any particular improvement in speed in lith emulsions containing vinyl polymers and ethyleneoxy polymers.

The addition of 3-pyrazolidone to the emulsion containing the onium salt, however, gives a very surprising increase in emulsion speed and this is enhanced further by some apparent synergism between the 3-pyrazolidone and an onium compound. The pyrazolidones used to advantage

include those disclosed in U.S. Pat. No. 2,751,297 and represented by the following general formula:



10 wherein X represents hydrogen or acetyl, R represents a heterocyclic group or an aryl group of the benzene or naphthalene series and R<sub>1</sub> represents hydrogen, an aryl group of the benzene or naphthalene series, or an alkyl group, and R<sub>2</sub> and R<sub>3</sub> each represents hydrogen or an alkyl group.

The following compounds are representative of the 3-pyrazolidone compounds useful in emulsions for the purposes of our invention:

- 20 1-phenyl-3-pyrazolidone  
1-p-tolyl-3-pyrazolidone  
5-phenyl-3-pyrazolidone  
5-methyl-3-pyrazolidone  
1-p-chlorophenyl-3-pyrazolidone  
25 1-phenyl-5-phenyl-3-pyrazolidone  
1-m-tolyl-3-pyrazolidone  
1-phenyl-5-methyl-3-pyrazolidone  
1-p-tolyl-5-phenyl-3-pyrazolidone  
1-m-tolyl-3-pyrazolidone  
30 1-p-methoxyphenyl-3-pyrazolidone  
1-p-acetamidophenyl-3-pyrazolidone  
1-phenyl-2-acetyl-4:4-dimethyl-3-pyrazolidone  
1-phenyl-4:4-dimethyl-3-pyrazolidone  
1-m-aminophenyl-4-methyl-4-n-propyl-3-pyrazolidone  
35 1-o-chlorophenyl-4-methyl-4-ethyl-3-pyrazolidone  
1-m-acetamidophenyl-4:4-diethyl-3-pyrazolidone  
1-(p-β-hydroxyethylphenyl)-4:4-dimethyl-3-pyrazolidone  
1-p-hydroxyphenyl-4:4-dimethyl-3-pyrazolidone  
40 1-p-methoxyphenyl-4:4-diethyl-3-pyrazolidone  
1-p-tolyl-4:4-dimethyl-3-pyrazolidone  
1-(7-hydroxy-2-naphthyl)-4-methyl-4-n-propyl-3-pyrazolidone  
1-p-diphenyl-4:4-dimethyl-3-pyrazolidone  
1-(p-β-hydroxyethylphenyl)-3-pyrazolidone  
45 1-o-tolyl-3-pyrazolidone  
1-o-tolyl-4:4-dimethyl-3-pyrazolidone  
1-benzothiazolyl-3-pyrazolidone  
4-methyl-1-phenyl-3-pyrazolidone

50 Useful concentrations of pyrazolidones in the photographic elements range from 0.005 to 2.0 gm./mole of silver in the emulsion. The preferred range is from 0.01 to 1.0 gm./mole of silver.

Optimum concentrations of the alkyleneoxy polymers and the pyrazolidones can be determined readily by actual tests in the emulsion and will vary with the formulation of the photographic emulsion and the developer used.

In general, both the alkyleneoxy polymer and the pyrazolidone are incorporated in the light-sensitive silver halide emulsion. While this is a particularly useful form of the invention, either or both the alkyleneoxy polymer and pyrazolidone may alternatively be present in an adjoining insensitive layer, or one or both can be imbibed from a processing bath, it being required only that both are present during development.

Our light-sensitive emulsions can be coated to advantage on any of the conventional photographic supports, including glass, cellulose acetate, polystyrene, polyalkyleneterephthalate, etc.

70 A typical lith-type developing solution which may be used contains as the only developing agent, hydroquinone or a hydroquinone derivative and having a very low sulfite ion content, the sulfite ion content being maintained by the presence in the solution of formaldehyde. "Lith-type" developing solutions are used for developing lithographic

film materials which contain photographic emulsions having an emulsion of uniform and fine-grain silver halide crystals. Such emulsions are developed in "lith-type" developing solutions to yield a contrast of 10 and above.

A typical "lith-type" developing solution is Kodak De-

The film samples were then fixed, washed and dried, and the speed, contrast, fog and dot quality evaluated. A dot quality scale from 1 to 10 represents increasing quality of half-tone dot with increasing number, 6 being a first acceptable quality of half-tone dot. The results are illustrated in Table I.

TABLE I

| Sample | 2 1/4 minutes developing time |                    |             |     | 3 1/4 minutes developing time |                    |             |     |
|--------|-------------------------------|--------------------|-------------|-----|-------------------------------|--------------------|-------------|-----|
|        | Relative speed                | Effective contrast | Dot quality | Fog | Relative speed                | Effective contrast | Dot quality | Fog |
| a----- | 100                           | 6.2                | 4 .01       |     | 102                           | 5.1                | 1 .01       |     |
| b----- | 46                            | 8.2                | 8 .01       |     | 65                            | 9.9                | 7 .01       |     |
| c----- | 48                            | 8.0                | 8 .01       |     | 68                            | 10.0               | 6 .01       |     |
| d----- | 50                            | 8.1                | 8 .01       |     | 69                            | 9.7                | 7 .01       |     |

veloper D-85 (see Kodak Formulas for the Graphic Arts, Kodak Pamphlet No. Q-11, p. 4) as follows:

#### KODAK DEVELOPER D-85

|                             |           |      |
|-----------------------------|-----------|------|
| Water about 90° F. (30° C.) | metric cc | 500  |
| Sodium sulfite desiccated   | grams     | 30.0 |
| Paraformaldehyde            | do        | 7.5  |
| Sodium bisulfite            | do        | 2.2  |
| Boric acid crystals         | do        | 7.5  |
| Hydroquinone                | do        | 22.5 |
| Potassium bromide           | do        | 1.6  |
| Water to make 1.0 liter.    |           |      |

The following examples are intended to illustrate our invention but not to limit it in any way:

#### EXAMPLE I

A high-contrast ortho-sensitized fine-grain gelatino chlorobromoiodide emulsion containing 90 mole percent silver chloride, 9 mole percent silver bromide, and ap-

20

It is shown that the addition of PEO, oleyl ether of polyethylene glycol having a molecular weight of 1540, raised contrast, dot quality, but caused speed loss. Further addition of Elon did not regain speed loss.

#### EXAMPLE II

Example I was repeated, except that the methyl-p-aminophenol was replaced by 4-methyl-1-phenyl-3-pyrazolidone as shown below:

- no further addition
- 0.5 gm. PEO, oleyl ether of polyethylene glycol having a molecular weight of 1540
- 0.5 gm. PEO, oleyl ether of polyethylene glycol having a molecular weight of 1540, plus .025 gm. 4-methyl-1-phenyl-3-pyrazolidone
- 0.5 gm. PEO, oleyl ether of polyethylene glycol having a molecular weight of 1540, plus .050 gm. 4-methyl-1-phenyl-3-pyrazolidone

30

35

The results are illustrated in Table II.

| Sample | 2 1/4 minutes developing time |                    |             |     | 3 1/4 minutes developing time |                    |             |     |
|--------|-------------------------------|--------------------|-------------|-----|-------------------------------|--------------------|-------------|-----|
|        | Relative speed                | Effective contrast | Dot quality | Fog | Relative speed                | Effective contrast | Dot quality | Fog |
| a----- | 100                           | 6.6                | 5 .01       |     | 112                           | 5.8                | 3 .01       |     |
| b----- | 48                            | 8.7                | 7 .01       |     | 68                            | 12.0               | 6 .01       |     |
| c----- | 68                            | 12.1               | 7 .01       |     | 83                            | 10.8               | 5 .01       |     |
| d----- | 87                            | 9.7                | 6 .01       |     | 102                           | 8.3                | 4 .01       |     |

proximately 1 mole percent silver iodide was prepared and split into separate portions. The following compounds were added to the individual portions in the indicated amounts per mole of silver halide:

- no further addenda
- 0.5 gm. PEO, oleyl ether of polyethylene glycol having a molecular weight of 1540
- 0.5 gm. PEO, oleyl ether of polyethylene glycol having a molecular weight of 1540 plus 0.025 gm. methyl-p-aminophenol
- 0.5 gm. PEO, oleyl ether of polyethylene glycol having a molecular weight of 1540 plus 0.050 gm. methyl-p-aminophenol

55

50

60

65

The various parts were coated on a cellulose triacetate film support at a coverage of 455 mg. of silver halide and 450 mg. of vehicle per square foot, dried, exposed to continuous and half-tone screen step wedges, developed for 2 1/4 minutes and 3 1/4 minutes, respectively, at a temperature of 68° F. in a developing solution of the following composition:

|                               |      |
|-------------------------------|------|
| Hydroquinone                  | 15.0 |
| Sodium formaldehyde bisulfite | 50.0 |
| Sodium bicarbonate            | 22.5 |
| Sodium carbonate              | 35.0 |
| Sodium sulfite                | 2.5  |
| Potassium bromide             | 0.75 |
| Water to make 1 liter.        |      |

It is shown that the addition of PEO, oleyl ether of polyethylene glycol having a molecular weight of 1540, raised contrast and dot quality but caused speed loss. Further addition of a 3-pyrazolidone regained speed, maintained contrast and dot quality.

#### EXAMPLE III

An emulsion was prepared as described in Example I. The following compounds were added to the individual portions in the indicated amounts per mole of silver halide.

- 0.03 gm. organosilicone, copoly(polyethyleneoxy-polypropyleneoxy-dimethylsiloxane), mol weight 2000, PPG-PEG 60-40, 9.5% by weight silicone
- 0.03 gm. organosilicone, copoly(polyethyleneoxy-polypropyleneoxy-dimethylsiloxane), mol weight 2000, PPG-PEG 60-40, 9.5% by weight silicone, plus 0.015 gm. 4-methyl-1-phenyl-3-pyrazolidone
- 0.03 gm. organosilicone, copoly(polyethyleneoxy-polypropyleneoxy-dimethylsiloxane), mol weight 2000, PPG-PEG 60-40, 9.5% by weight silicone, plus 5.0 gm. hydroquinone. Each sample was processed and evaluated as in Example I. The results are shown in Table III.

TABLE III  
[DEVELOPING TIME: 1½ MINUTES]

| Sample: | Relative speed | Effective contrast |
|---------|----------------|--------------------|
| a-----  | 100            | .55                |
| b-----  | 741            | 6.3                |
| c-----  | 289            | 2.4                |

It is shown that the addition of 4-methyl-1-phenyl-3-pyrazolidone has considerably increased contrast, while the addition of hydroquinone has not.

## EXAMPLE IV

An emulsion was prepared as in Example I wherein the vehicle comprised, per mole of silver halide, 46 gm. of gelatin and 92 gm. of copoly(butyl acrylate-acrylic acid-4,4,9-trimethyl-8-oxo-7-oxa-4-azonia-9-decene - 1 - sulfonate). The emulsion was split into two portions, one of which was retained as a control. To the other portion was added, per mole of silver halide, 0.015 gm. of 4-methyl-1-phenyl-3-pyrazolidone. Each sample was processed and evaluated as in Example I. The results are shown in Table IV.

TABLE IV  
[DEVELOPING TIME: 2½ MINUTES]

| Sample:                                                 | Relative speed | Effective contrast |
|---------------------------------------------------------|----------------|--------------------|
| Control-----                                            | 194            | 5.4                |
| Sample containing 4-methyl-1-phenyl-3-pyrazolidone----- | 253            | 11.2               |

Result: 4-methyl-1-phenyl - 3 - pyrazolidone has increased speed and contrast.

## EXAMPLE V

An emulsion was prepared as in Example IV and split into two portions, (a) and (b). To each portion were added, per mole of silver halide, .030 gm. of organosilicone, copoly(polyethyleneoxypropyleneoxy - dimethylsiloxane), mol weight 2000, PPG-PEG 60-40, 9.5% by weight silicone. To portion (b) was added, in addition, .015 gm. of 4-methyl-1-phenyl-3-pyrazolidone per mole of silver halide. Each sample was processed and evaluated as in Example I. The results are shown in Table V.

TABLE V  
[DEVELOPING TIME: 1½ MINUTES]

| Sample: | Relative speed | Effective contrast |
|---------|----------------|--------------------|
| a-----  | 100            | 3.5                |
| b-----  | 661            | 8.2                |

Result: The 3-pyrazolidone has increased speed and contrast.

## EXAMPLE VI

An emulsion was prepared as in Example IV and split into two portions, (a) and (b). To each portion were added, per mole of silver halide, 0.100 gm. of an organosilicone, a water-soluble polysiloxane made up of dimethyl silicone sections and polyether sections and containing 6.5% by weight of silicone, and .5 gm. of  $\omega$ -hydroxydecyl pyridinium-perchlorate. To portion (b) were added, in addition, .015 gm. of 4-methyl-1-phenyl-3-pyrazolidone. Each sample was processed and evaluated as in Example I. The results are shown in Table VI.

TABLE VI.—DEVELOPING TIME: 2 MINUTES

| Sample: | Relative speed | Effective contrast |
|---------|----------------|--------------------|
| a-----  | 208            | 1.6                |
| b-----  | 266            | 10.0               |

Result: Addition of an onium salt, a known developer accelerator, has given acceptable speed, but has lowered contrast. Addition of 4-methyl-1-phenyl-3-pyrazolidone has improved speed further and given excellent contrast.

10  
EXAMPLE VII

This is a repeat of Example VI, except that Sample (a) contained only 0.085 gm. of the organosilicone of Example VI.

The results are shown in Table VII.

TABLE VII.—DEVELOPING TIME: 2 MINUTES

| Sample: | Relative speed | Effective contrast |
|---------|----------------|--------------------|
| a-----  | 100            | 2.2                |
| b-----  | 229            | 7.0                |

Results: Same as in Example VI.

## EXAMPLE VIII

An emulsion was prepared as in Example IV and split into three portions, (a), (b), and (c). To portion (a) were added per mole of silver halide, .025 gm. of a block copolymer of polyethyleneoxide and polypropyleneoxide units having a total molecular weight of 2000 and wherein the molecular weight of the polypropyleneoxide constituent is 1200 and wherein the ratio by weight of the polyethyleneoxide to polypropyleneoxide is 60 to 40; to portion (b), .025 gm. of a polymer similar to (a) above, having a total molecular weight of 2920 and wherein the molecular weight of the polypropyleneoxide constituent is 1750 and wherein the ratio by weight of the polyethyleneoxide to polypropyleneoxide is 40 to 60; to portion (c), .055 gm. of a polypropyleneoxide-polyethyleneoxide glutarate having a total molecular weight of 2000 and wherein the ratio by weight of polyethyleneoxide to polypropyleneoxide is 60 to 40 and wherein the polypropylene constituent has a molecular weight of 1200. To each portion were added, in addition, .015 gm. of 4-methyl-1-phenyl-3-pyrazolidone and .3 gm. of  $\omega$ -hydroxydecyl pyridinium-perchlorate. Each sample was processed and evaluated as in Example I. The results are shown in Table VIII.

TABLE VIII.—DEVELOPING TIME: 2 MINUTES

| Sample: | Relative speed | Effective contrast |
|---------|----------------|--------------------|
| a-----  | 110            | 6.0                |
| b-----  | 107            | 6.5                |
| c-----  | 100            | 7.0                |

Result: All coatings showed excellent speed and good contrast.

## EXAMPLE IX

An emulsion was prepared as in Example I wherein the vehicle comprised, per mole of silver halide, 70 gm. of gelatin and 70 gm. of copoly(butyl acrylate-acrylic acid-4,4,9 - trimethyl - 8-oxo-7-oxa-4-azonia-9-decene-1-sulfonate). The emulsion was split into two portions, (a) and (b). To each portion were added, per mole of silver halide, .075 gm. of the block polymer A of Example VIII and .500 gm. of  $\omega$ -hydroxydecyl pyridinium-perchlorate. To portion (b) were added, in addition, .015 gm. of 4-methyl-1-phenyl-3-pyrazolidone. Each sample was processed and evaluated as in Example I. The results are shown in Table IX.

TABLE IX.—DEVELOPING TIME: 2½ MINUTES

| Sample: | Relative speed | Effective contrast |
|---------|----------------|--------------------|
| a-----  | 100            | .22                |
| b-----  | 646            | 11.2               |

The advantageous effect of the 3-pyrazolidone with respect to speed and contrast is retained when the vinyl polymer concentration in the emulsion vehicle is increased to constitute 50 percent of the total vehicle.

## EXAMPLE X

To an emulsion as described in Example I were added, per mole of silver halide, 0.1 gm. of organosilicone block polymer of Example VI. The emulsion was then divided into two portions, A and B. To portion B were added,

per mole of silver halide, 0.015 gm. of 4-methyl-1-phenyl-3-pyrazolidone. After coating, the above portions of emulsion as described in Example I, samples of each film were processed as described in Example I at the developing times as shown below: the results are listed in Table X.

TABLE X

| Coating No.: | Portion A         |                |                    |             |
|--------------|-------------------|----------------|--------------------|-------------|
|              | Developing time   | Relative speed | Effective contrast | Dot quality |
| 1-----       | 1 $\frac{3}{4}$ ' | 100            | 6.5                | 8           |
| 2-----       | 2 $\frac{3}{4}$ ' | 195            | 10.5               | 8           |
| 3-----       | 3 $\frac{3}{4}$ ' | 324            | 13.5               | 8           |
| 4-----       | 4 $\frac{3}{4}$ ' | 513            | 16.0               | 7           |

  

| Coating No.: | Portion B         |                |                    |             |
|--------------|-------------------|----------------|--------------------|-------------|
|              | Developing time   | Relative speed | Effective contrast | Dot quality |
| 5-----       | 1 $\frac{3}{4}$ ' | 115            | 6.5                | 8           |
| 6-----       | 2 $\frac{3}{4}$ ' | 240            | 11.5               | 9           |
| 7-----       | 3 $\frac{3}{4}$ ' | 398            | 13.0               | 9           |
| 8-----       | 4 $\frac{3}{4}$ ' | 603            | 16.0               | 8           |

It is shown that the addition of small amounts of 4-methyl-1-phenyl-3-pyrazolidone to silver halide emulsions containing polyalkylene oxide-dialkyl siloxane polymers results in an increase in speed, contrast and halftone dot quality over a wide range of developing time.

## EXAMPLE XI

One film sample of each coating made with emulsion portions A and B of Example X was incubated for 1 week at 120° F. and 50% relative humidity. Each of the incubated samples was, together with a nonincubated corresponding sample, immersed at a temperature of 68° F. for 4 minutes into a developing solution of the following composition:

|                                     |     |      |
|-------------------------------------|-----|------|
| Water -----                         | ml. | 500  |
| Methyl-p-aminophenol -----          | gm. | 1.0  |
| Sodium sulfite, dessicated -----    | gm. | 75.0 |
| Hydroquinone -----                  | gm. | 9.0  |
| Sodium carbonate, monohydrate ----- | gm. | 30.0 |
| Potassium bromide -----             | gm. | 5.0  |
| Water to make 1.0 liter.            |     |      |

The observed fog of each sample is recorded in Table XI.

TABLE XI

| Coating: | Fog        |                  |
|----------|------------|------------------|
|          | Fresh test | Incubated sample |
| A-----   | .12        | .34              |
| B-----   | .12        | .12              |

It is shown that the presence of 4-methyl-1-phenyl-3-pyrazolidone has effectively protected the film material against fog growth upon incubation.

## EXAMPLE XII

This example illustrates the advantageous synergistic effect with respect to the contrast obtainable with a combination of polypropylene glycol copolymer and a 3-pyrazolidone in a lith-type emulsion. To each of three different portions of an emulsion as described in Example I were respectively added, per mole of silver halide, (a) 0.025 gm. of block polymer A of Example VIII, (b) 0.025 gm. of block polymer A of Example VIII, plus 0.015 gm. 4-methyl-1-phenyl-3-pyrazolidone, (c) 0.015 gm. 4,4-dimethyl-1-phenyl-3-pyrazolidone.

Each sample was processed according to the procedure of Example I. The results are recorded in Table XII.

TABLE XII

| Coating: | Developing time, min. | Relative speed |      | Effective contrast |
|----------|-----------------------|----------------|------|--------------------|
|          |                       | 100            | 186  |                    |
| a-----   | 2                     | 100            | 7.5  | 7.5                |
| b-----   | 2                     | 115            | 10.5 | 10.5               |
| c-----   | 2                     | 186            | 9.0  | 9.0                |

12  
EXAMPLE XIII

This example illustrates the advantage derived from the presence of the pyrazolidone in the emulsion over its presence in the developer solution. It also illustrates, again, the superiority of a pyrazolidone over other common developing agents as an addenda in the lith-type materials of our invention.

Several film strips were prepared according to the procedures described in the preceding examples. They comprised, in addition to silver halide and other common addenda, the following compounds per mole of silver halide:

| Strip: | Block polymer<br>A of Example<br>VIII, grams | Developer                                      |                       |
|--------|----------------------------------------------|------------------------------------------------|-----------------------|
|        |                                              | 4-methyl-1-phenyl-3-pyrazolidone,<br>0.015 gm. | Hydroquinone, 0.5 gm. |
| A----- | 0.025                                        | None                                           |                       |
| B----- | 0.025                                        |                                                |                       |
| C----- | 0.025                                        |                                                |                       |
| D----- | 0.025                                        |                                                |                       |

Strips A, B, and C were developed in the developer solution of Example I. Strip D was developed in the developer solution of Example I to which were added 5 gm. of 4-methyl-1-phenyl-3-pyrazolidone per liter of solution. The development time was in each case 1 $\frac{3}{4}$  minutes.

| Strip: | Relative speed | Effective contrast |    | Dot quality | Fog |
|--------|----------------|--------------------|----|-------------|-----|
|        |                | 100                | 89 |             |     |
| A----- | 100            | 9.4                | 8  | .01         |     |
| B----- | 89             | 6.9                | 5  | .02         |     |
| C----- | 93             | 7.7                | 6  | .02         |     |
| D----- | 85             | 7.3                | 6  | .02         |     |

“Effective Contrast” of a developed photographic material differs from the conception of “contrast” which is in the photographic art generally synonymous with only the slope of the straightline portion of the characteristic curve, in that the slope of the characteristic curve in the toe region is also taken into account. For example, two different photographic materials may exhibit identical contrasts, but the one whose characteristic curve shows also a more acute shape of the curve in the toe region has a higher effective contrast.

Other tests similar to those described above have shown (a) that coatings of lith-type emulsions containing a vinyl polymer for the purpose of improving dimensional stability require a considerably longer development time to yield satisfactory dot quality than coatings not containing such vinyl polymers and that at such prolonged development times the vinyl polymer containing coatings produced unacceptably high fog, (b) materials as described under (a) which, in addition, contained a 3-pyrazolidone did not exhibit the cited undesirable side effects introduced by the vinyl polymer.

The quality of the silver images produced in “lith-type” emulsion layers is conveniently measured in terms of effective contrast and dot quality. Dot quality is a measure of the quality of the reproduction of a half-tone image “lith-type” photographic elements exposed to a half-tone image, and developed, produce areas commonly referred to as shadow dots and areas known as highlight areas. Intermediate between these two extremes are areas of varying size. The dot quality used herein is a measure of the areas referred to as 50% dots (i.e.,  $\frac{1}{2}$  clear, and  $\frac{1}{2}$  developed density) and is expressed in a progressive scale where “9” is excellent and “1” is extremely poor. A 50% dot quality below “6” is generally not acceptable.

The beneficial combination of addenda which constitutes our invention are used to particular advantage in lith emulsions containing more than 50 mole percent of silver chloride. The image reproductions produced in our lithographic emulsion layers are of excellent quality. Although the conventional alkaline, pure hydroquinone, low free-sulfite developer may be used to develop these exposed elements, it is also advantageous to use a pure hydroquinone developer having from 10 to about 30 grams of an alkali-sulfite per liter of developing solution or even an Elon-hydroquinone developer having from 10 to about 30 grams of an alkali-sulfite per liter of developing solution. When the elements of this invention are developed in one of the two latter developing solutions, not only is the image contrast high and the dot quality excellent, but this excellent quality is produced over a wide range of exposure and development times.

Typical polymeric vinyl compounds useful in our invention are disclosed in U.S. Pat. 3,142,568, issued July 28, 1964, incorporated herein by reference.

The invention has been described in detail with particular reference to preferred embodiments thereof, but it will be understood that variations and modifications can be effected within the spirit and scope of the invention as described hereinabove and as defined in the appended claims.

We claim:

1. A light-sensitive photographic element comprising a support having thereon at least one light-sensitive silver halide emulsion in which the chloride comprises at least 50 mole percent of the halide, containing a hydrophilic colloid binder, a polyalkyleneoxy polymer in amount of about 0.01 gram to about 3.0 grams per mole of silver halide, and a 3-pyrazolidone silver halide developing agent in an amount of about 0.005 gram to about 2.0 grams per mole of silver halide.

2. A photographic element of claim 1 in which the colloid binder is gelatin.

3. A light sensitive photographic element of claim 2 containing an onium salt.

4. A light sensitive photographic element of claim 2 containing an aqueous dispersion of a polymerized vinyl compound.

5. A light sensitive photographic element of claim 2 comprising an aqueous dispersion of a polymerized vinyl compound and an onium salt.

6. A light sensitive photographic element of claim 2 in which said support is a dimensionally stable polymeric support and said element comprises an aqueous dispersion of a polymerized vinyl compound and an onium salt.

7. A photographic element of claim 4 in which the ratio of gelatin to vinyl polymer ranges from 20 to 80 to 80 to 20 parts by weight.

8. A photographic element of claim 4 in which the vinyl polymer comprises an acrylic acid-ester polymeric compound selected from the group consisting of a homopolymer of an acrylic acid-ester and a copolymer of acrylic acid-ester and acrylic acid, said copolymer containing at least 80% by weight of units of said acrylic acid esters.

9. A photographic element of claim 4 in which the vinyl polymer comprises an interpolymer selected from the group consisting of acrylic acid, unsaturated carboxylic acid esters and sulfobetaines, said interpolymer containing (1) up to about 15% by weight, of acrylic acid, (2) at least about 75%, by weight of a monomer having the formula:



wherein R is hydrogen or methyl and R<sub>1</sub> is an alkyl radi-

cal, containing 1-12 carbon atoms, with (3) up to about 10%, by weight, of a monomer having the formula:



wherein R is hydrogen or alkyl, R<sub>1</sub> and R<sub>4</sub> are each divalent saturated aliphatic hydrocarbon radicals, containing up to 12 carbon atoms, and R<sub>2</sub> and R<sub>3</sub> are each hydrogen or alkyl.

10. A photographic element of claim 1 in which the polyalkyleneoxy polymer is the oleyl ether of polyethylene glycol.

11. A photographic element of claim 1 in which the polyalkyleneoxy polymer is a block polymer of polyoxypropylene and polyoxyethylene represented by the formula:



wherein Y represents an organic radical having a valence of x; n is an integer; x is an integer greater than 1, so that the values of n and x are such that the molecular weight of the said polymer exclusive of Y, E and R is between 800 and 3,000; E represents a polyoxyethylene chain constituting from about 10 to about 70 percent by weight of said polymer; and R is a member selected from the class consisting of the hydrogen atom, an alkyl group, an alkyl carbonyl group, and an aryl carbonyl group.

12. A photographic element of claim 1 in which the polyalkyleneoxy polymer is a block copolymer of polyoxypropylene and polyoxyethylene represented by the formula:



35 wherein b represents an integer of from 14 to 52; and a and c each represent integers such that the sum of a+c represents an integer of from 4 to 48 and the polyoxyethylene groups constitute between 10 and 70 percent by weight of said polymer.

13. A photographic element of claim 11 in which the copolymer of polyoxypropylene and polyoxyethylene contains in the main chain silicone atoms at concentration ranges up to approximately 15% by weight, of the polymer compound.

45 14. A photographic element of claim 12 in which the copolymer of polyoxypropylene and polyoxyethylene contains in the main chain silicone atoms at concentrations ranging up to approximately 15%, by weight, of the polymer compound.

50 15. A photographic element of claim 3 in which the onium salt is selected from the class consisting of a quaternary ammonium salt, a sulfonium salt and a phosphonium salt.

55 16. A photographic element of claim 3 in which the concentration of the onium salt ranges from approximately 0.01 to approximately 2.0 grams per mole of silver halide in the emulsion.

60 17. A photographic element of claim 1 in which the 3-pyrazolidone is selected from the class represented by the following generic formula:



wherein X represents hydrogen or acetyl, R represents a heterocyclic group or an aryl group of the benzene or naphthalene series and R<sub>1</sub> represents hydrogen, an aryl group of the benzene or naphthalene series, or an alkyl group, and R<sub>2</sub> and R<sub>3</sub> each represents hydrogen or an alkyl group.

75 18. A photographic element of claim 4 in which the

ratio of gelatin to vinyl polymer ranges from 20 to 80 to 80 to 20 parts by weight.

19. A photographic element of claim 5 in which the polymerized vinyl compound comprises an acrylic acid-ester polymeric compound selected from the group consisting of a homopolymer of an acrylic acid-ester, and a copolymer of acrylic acid-ester and acrylic acid, said copolymer containing at least 80% by weight of units of said acrylic acid-esters.

20. A photographic element of claim 5 in which the polymerized vinyl compound comprises an interpolymer selected from the group consisting of acrylic acid, unsaturated carboxylic acid-ester and sulfobetaines, said interpolymer containing (1) up to about 15%, by weight, of acrylic acid, (2) at least about 75%, by weight, of a monomer having the formula:



wherein R is hydrogen or methyl and R<sub>1</sub> is an alkyl radical, containing 1-12 carbon atoms, with (3) up to about 10%, by weight, of a monomer having the formula:



wherein R is hydrogen or alkyl, R<sub>1</sub> and R<sub>4</sub> are each divalent saturated aliphatic hydrocarbon radicals, containing up to 12 carbon atoms and R<sub>2</sub> and R<sub>3</sub> are each hydrogen or alkyl.

21. A photographic element of claim 15 in which the concentration of said polyethylenoxy polymer present in said emulsion ranges from 0.001 to 3.0 grams per mole of silver halide.

22. A photographic element of claim 15 in which the polyalkylenoxy polymer is the oleyl ether of polyethylene glycol.

23. A process of developing an exposed photographic silver halide emulsion in which the halide comprises at least 50 mole percent chloride, comprising imbibing into the said emulsion about 0.01 gram to 3.0 grams per mole of silver halide of a polyalkylenoxy polymer and about 0.005 gram to about 2.0 grams per mole of silver halide of a 3-pyrazolidone silver halide developing agent, and reducing the exposed silver halide to silver.

#### References Cited

##### UNITED STATES PATENTS

|    |           |         |                |       |           |
|----|-----------|---------|----------------|-------|-----------|
| 20 | 3,017,271 | 11/1962 | Piper          | ----- | 96-66.3 X |
|    | 3,142,568 | 7/1964  | Nottorf        | ----- | 96-87     |
|    | 3,158,483 | 11/1964 | Lowe et al.    | ----- | 96-66.3   |
|    | 3,312,550 | 4/1967  | Stewart et al. | ----- | 96-76 X   |
|    | 3,294,540 | 12/1966 | Goffe          | ----- | 96-107    |

25 NORMAN G. TORCHIN, Primary Examiner

R. E. FICHTER, Assistant Examiner

U.S. CL. X.R.

30 96-65, 107, 109, 114